

## UNITED STATES PATENT OFFICE.

EDOUARD M. KRATZ, OF CHICAGO, ILLINOIS, ASSIGNOR TO MARSENE PRODUCTS CO., OF CHICAGO, ILLINOIS, A CORPORATION OF ILLINOIS.

## METHOD OF FORMING GELATIN SHEETS AND SURFACES THEREFOR.

No Drawing. Application filed February 24, 1925, Serial No. 11,335. Renewed January 7, 1929.

This invention relates to a particular type of prepared surface for the formation of transparent paper of gelatin composition thereon.

5 Hitherto various surfaces have been known and used for forming such sheets. Among the various ones are polished stone or matrix surfaces, metallic surfaces such as zinc, and surfaces formed from cellulose esters, such as 10 nitro-cellulose, cellulose acetate, etc. These surfaces all have their disadvantages. The stone surfaces have but a limited use. The metallic surfaces are apt to corrode and form other blemishes that result in imperfect gelatin sheets. The cellulosic surfaces are apt 15 to be fragile and to crack when folded or to mar easily. Such surfaces, especially when formed of nitro-cellulose or pyroxyline materials, have a tendency to cause gelatin sheets 20 containing softening oils to become milky or cloudy due to the action of the nitro-cellulose materials on the softening oils. Moreover, difficulty is often experienced in stripping the finished gelatin from any of the above surfaces due to a tendency of the sheet to adhere 25 to the surface.

It is an object of this invention to provide a prepared surface of durable qualities upon which to form gelatin sheets and from which 30 such sheets may be easily stripped.

It is a further object of this invention to provide a prepared surface suitable for use in combination with a flexible base that will have good flexible and folding qualities.

35 Other and further important objects of this invention will be apparent from the disclosures in the specification and the appended claims.

While the prepared surface may be used 40 in conjunction with a rigid base, as on a flat table surface, I prefer to use it in conjunction with a flexible endless belt, since this use is best adapted for production purposes.

The surface which I have found best adapted 45 for use in forming gelatin sheets is that afforded by a waterproof coating for textiles, consisting largely of linseed oil and other blended oils. The fabric used as a base for this surface is a thin English muslin which 50 has been bleached, shrunk and dyed. To this

muslin fabric are applied by means of a doctor, base coats of pigments suspended in drying oils. The coated fabric is then festooned and baked at 180° F. Extra care must be taken to see that the first coat applied to the 55 fabric is properly anchored. The fabric is then calendered to smooth out the surface. Successive base coats are applied until a relatively smooth surface is obtained. Then several coats of linseed and other blended oils are 60 applied by means of a doctor, and between each successive coat the material is festooned and baked, until a perfectly smooth glazed surface is obtained. The oils used for glazing are centrifuged or filtered to remove any 65 foreign matter that might cause pimples or other rough places in the finished surface. This surface is now smooth, durable, has excellent folding qualities and is not easily cracked. On account of the thinness of the 70 fabric, it has the property of contracting with the gelatin sheet as the gelatin sheet contracts. This results in a denser, stronger sheet than would be possible if a rigid, non-contracting base were used, since in this latter case the gelatin sheet has a tendency to pull away from 75 the base in contracting during the drying, and thus to weaken the sheet through the internal stresses set up by the contraction of the gelatin.

However, the surface need not be smooth but may be impressed with any desired design, since the qualities of the coating are such that there is no tendency of the gelatin sheet to stick to the surface during the stripping process. If a coating having a stamped design is used, the design is faithfully reproduced on the gelatin sheet.

The methods of forming the gelatin sheets on such a prepared surface as above described 90 are many, but I prefer to use the surface in connection with the process and apparatus described in my copending application for "transparent paper and a process of manufacture", S. N. 10,962, filed February 21, 1925. 95 According to that process, a gelatin composition comprising approximately 60% to 85% glue and 15% to 40% sulphonated castor oil is employed.

In connection with suitable apparatus a 100

warm gelatin sulphonated oil composition solution is applied to an endless belt made from the fabric material having this prepared surface. After the gelatin film has been jelled and dried to harden it, it is stripped from the surface by any suitable means. The stripping process is much more satisfactory than hitherto when other surfaces were used. In this way and with this prepared surface, very thin, perfectly clear, unblemished gelatin sheets may be prepared.

I am aware that many changes may be made, and numerous details of the method may be varied through a wide range without departing from the principles of this invention, and I therefore do not purpose limiting the patent granted hereon, otherwise than necessitated by the prior art.

I claim as my invention:

- 20 1. A surface for forming gelatin sheets containing sulphonated oil, largely comprised of linseed oil and other blended oils.
- 25 2. The method of preparing sheets of gelatin-sulphonated oil composition, comprising spreading a solution of said composition over a surface comprising a preparation of linseed oil and other blended oils, cooling such solution to allow the composition to jell, drying and then stripping the sheet so formed from such surface.
- 30 3. The method of preparing gelatin sheets containing sulphonated oil, comprising applying a gelatin and sulphonated oil solution to a surface comprising largely a preparation of drying oils, allowing the solution to harden, drying and then stripping the sheet so formed from said surface.
- 35 4. In combination with a machine for making transparent paper of gelatin and sulphonated oil composition, a sheet forming surface comprising a web of thin fabric material having a coating of baked drying oils adhering thereto.
- 40 5. Web material for use in the formation of gelatin composition, transparent sheets, comprising a fabric having a coating thereon of baked drying oils on which said sheets may be formed and from which said sheets may be readily stripped when dry.
- 45 50 In testimony whereof I have hereunto subscribed my name.

EDOUARD M. KRATZ.